

## UNITED STATES PATENT OFFICE

2,322,968

## DYEING PANAMA HATS

George M. Rickus, William L. Braun, and Stanley G. Hoffman, Norwalk, Conn., assignors to Hat Corporation of America, Norwalk, Conn., a corporation of Delaware

No Drawing. Application May 4, 1940,  
Serial No. 333,424

7 Claims. (Cl. 8—3)

This invention relates to palm fibers, and to the process of dyeing palm fibers. An important application of the present invention is in the Panama hat industry.

It has been customary to manufacture Panama hat bodies in foreign countries. Bruises ordinarily develop during the weaving of the hat bodies from the palm fiber. Partly to make the bruised spots less noticeable, it has been customary to pound the fibers and to rub sulfur into them. The hats have ordinarily been shipped in a folded condition, and bruises have developed during shipment. Hats are conventionally bleached at bleacheries, and shipped to hat factories for finishing operation.

Several methods of dyeing Panama hats have been tried in the past. None of the processes have been satisfactory. Dyed Panama hats have been objectionable because:

(1) There has been little penetration of the dye. The dyeing process has been almost a surface coating. Whenever a fiber has been abraded or broken, as for example in handling, the cross-section has shown the ring of surface dyeing and a center of undyed palm.

(2) There has been too little flexibility, and too much brittleness. Dyed Panama fibers have been both weak and fragile.

(3) There has been a lack of uniformity of color distribution, because the dyeing processes have affected bruised and unbruised portions differently, and because the dyestuffs inherently produced some shading.

Accordingly, it is an important object of the present invention to provide as a new product a dyed Panama hat having little brittleness and the general physical characteristics of an undyed hat.

Another object is to provide a process by means of which the dye is made to penetrate throughout the fiber, so that if the hat becomes bruised or cut, the cross-section of the fiber will show approximately the same uniform color throughout.

A further object is to provide a method of dyeing palm fibers which will give a substantially uniform color to both the bruised and unbruised portions of the fiber.

Another object is to provide a manufacturing process minimizing the bruising of the fibers of a Panama hat.

Yet another object is to provide a process giving uniform distribution of color upon a Panama hat or like article.

A still further object is to provide a dyeing process adapted to dye unbleached and semi-bleached, as well as bleached Panama hats.

Another object is to provide a process by means of which the reflection of light from a dyed Panama hat is more accurately controlled.

Another object is to provide a process for making waterproofed fibers.

A feature resulting in the attainment of the foregoing objects is the use of a dyeing solution containing dyestuffs chosen from each of two classes of dyestuffs.

5 Another feature is the control of the temperature of the dyeing solution to effect a more thorough distribution and uniform penetration of the color.

Other features include:

10 The use of a wetting out process to make the palm fibers more susceptible to the penetration of the color.

The use of an emulsifying agent to stabilize a suspension of a water insoluble dye.

15 The use of a lacquer on the Panama hats to control the reflection of light from the hat.

The use of a process of preparing, shipping, and bleaching unfinished Panama hat bodies without extensively bruising the same.

20 Other objects and features can be appreciated upon reading the detailed description and claims hereinafter.

The detailed description which follows is under various headings to facilitate an understanding 25 of the process and the article of manufacture. The present invention is not limited to the details described herein, for the invention is capable of other methods of operation. Therefore, the phraseology used is for the purpose of description and not of limitation.

## PREPARING UNFINISHED HAT BODIES

According to the present invention Panama hat bodies, woven with the minimum amount of 35 bruising, are shipped as untrimmed bodies. Ordinarily hat bodies are pounded, and treated with sulfur, but according to the process of the present invention, the Panama hat bodies are given as little bruising as possible, and no sulfur is rubbed or pounded into the fibers at any time.

40 Preferably the untrimmed hats are shipped with the crown of each hat inside the crown of the hat above it. Because they are untrimmed hats, there is little possibility of bruising either the brim or the crown.

45 Before being bleached the untrimmed sulfur-free hat bodies are given a preliminary blocking. An ordinary bleaching solution has been found satisfactory. Better results are obtained with the dyeing process of the present invention in

50 dyeing unbleached hats than has heretofore been possible with unbleached hats. With certain dyestuffs, better results are obtainable with semi-bleached hat bodies than with bleached hat bodies. Ordinarily, however, it is best to bleach the hat bodies. Regardless of how many precautions are taken, however, it has been found commercially impossible to prepare a completely unbruised hat for a dye bath, but if the procedure

outlined above is followed the amount of bruising is minimized.

#### WETTING OUT

The preferably untrimmed, sulfur free, blocked, and bleached Panama hat bodies are then placed in water to effect a thorough wetting of the fibers. Panama hat workers can readily determine whether the fibers are thoroughly wetted by the feel of the material. If the fibers are immersed for an unduly prolonged time, they are so soft as to be very easily bruised, and if they are not thoroughly wetted, the penetration of the dye is not as complete and/or as rapid as desired. The exact period of time necessarily varies according to the prior treatment of the hat, the diameter of the fiber, and many other variables, but can be easily determined for each batch by a person skilled in the art. Whether semibleached hat bodies, unbleached hat bodies, raw palm fiber, or equivalent materials are to be dyed, they are subjected to a thorough wetting out process, sufficient to penetratingly soak the material, but insufficient to make the material exceptionally susceptible to bruising.

Soaking the hats in water for twelve hours at a temperature of 50 to 70° F. has been found to be satisfactory, as has soaking in a water solution containing one-tenth of one per cent of Nekal NS (sodium sulfonate of a fatty acid ester), at 100° F., for five hours. Instead of using Nekal NS, Peregol O (ethylene oxide condensate with higher fatty alcohol), Naconal NR (sodium alkylarylsulfonate), Gardinol (sodium sulfate of technical oleyl alcohol), Clarol, Decersol OT (sodium salt of dioctylsulfosuccinate), Sulframine DRX, or an equivalent wetting agent may be used.

#### PREPARATION OF DYE LIQUOR

According to the present invention, a dyeing solution is used which contains at least one of each of two classes of dyestuffs. It has been found that certain kinds of dyestuffs will dye the bruised fibers, and that certain other kinds of dyestuffs will dye the unbruised fibers. It has also been found that a dye bath containing at least one of each class of dyestuff will satisfactorily dye a somewhat bruised Panama hat. It is possible to produce a hat having the same shade upon both the bruised and the unbruised portions, or having shades so nearly the same that the difference cannot be normally detected. However, the bruised and unbruised portions reflect light differently, and the bruised spots in the dyed but unfinished hat can sometimes be detected by means of the differences in reflection of light. To obtain most satisfactory results, therefore, it is desirable that the hats, prior to the dyeing operation, be treated and handled in a manner to minimize bruising.

The class of dyestuffs satisfactorily dyeing the unbruised portion of the fibers hereinafter sometimes designated as "class A dyestuffs" has been found to include two kinds, namely: acetate dyestuffs; and spirit or oil soluble dyestuffs. Acetate dyestuffs are insoluble in but dispersible in water, and were originally developed for dyeing acetate rayon. Acetate dyestuffs are known by that name in the trade. Similarly spirit or oil soluble dyestuffs include those which are soluble in either oil or spirit, and are known to the trade by that name. In referring to oil or spirit soluble dyestuffs those appreciably soluble in any of the organic solvents, including or similar to min-

eral oil, ethyl alcohol, glycol, butyl acetate, Cellosolve, Carbitol, etc. are meant to be included.

Among the class A dyestuffs that have been found satisfactory are Celliton Fast Yellow GA, 5 Cibacet Red B, Celliton Fast Blue FR, Celliton Fast Pink RF, Celliton Fast Orange R, Ciba Orange 3R, Celliton Fast Blue Green B, Celliton Fast Blue FFC, Azosol Fast Red BB, and Azosol Fast Red 3B.

The class of dyestuffs satisfactorily dyeing the bruised portion of the fibers, hereinafter sometimes designated as "class B dyestuffs" has been found to include two kinds, namely: direct dyestuffs; and neutral dyeing acid dyestuffs.

Among the class B dyestuffs that have been found satisfactory are Brilliant Indocyanine G, Brilliant Wool Blue FFB Ex (Prototype 40), Fastusol Yellow 2G (Rowe's C. I. 346), Brilliant Pure Yellow 6 GS Conc. (Rowe's C. I. 802), Benzo Rhoduline Red B (Schultze C. I. 305), Benzo Orange R Conc. New, Diamini Brown 3 GTA, Azo Fast Yellow CGG, Azosol Fast Violet BB, Fastusol Red 4 BA, Fastusol Red L5B, Azosol Fast Blue LRA, Fastusol Pink G, and Fastusol Red 5B.

All of said class A and class B dyestuffs can be purchased through General Dyestuffs Corporation, New York city.

At least one class A dyestuff is mixed with Gardinol, or an equivalent emulsifying agent, and then dispersed in boiling water. To this suspension is added at least one class B dyestuff, and enough water is added to dissolve the class B dyestuff. Those skilled in the art are accustomed to preparing pastes of this nature by similar procedures. The ratio of class A to class B dyestuff is dependent partly upon the relative proportion of bruised to unbruised fibers to be dyed, but even more dependent upon the depth of shade desired. The degree of matching of shades also effects the A:B ratio.

If eighteen Panama hats weighing approximately 990 gms. are to be dyed a canary yellow, a dyeing paste may be made up as follows:

|                       | Grams |
|-----------------------|-------|
| Celliton Yellow GA    | 4.455 |
| Ciba Orange 3R        | 1.485 |
| Celliton Blue Green B | .128  |

|    |                         |       |
|----|-------------------------|-------|
| 50 | Total class A dyestuffs | 6.068 |
|----|-------------------------|-------|

|    |                        |       |
|----|------------------------|-------|
| 55 | Fastusol Yellow 2G     | 3.465 |
|    | Brill Pure Yellow 6 GS | 2.970 |
|    | Benzo Rhoduline        | .297  |

|    |                         |       |
|----|-------------------------|-------|
| 60 | Total class B dyestuffs | 6.732 |
|----|-------------------------|-------|

|    |                 |        |
|----|-----------------|--------|
| 65 | Total dyestuffs | 12.800 |
|----|-----------------|--------|

If thirteen hats weighting approximately 685 gms. are to be dyed a roseleaf pink, a dyeing liquor may be made up as follows:

|    | Grams                 |       |
|----|-----------------------|-------|
| 65 | Celliton Fast Pink RF | 6.596 |
|    | Celliton Yellow GA    | 1.933 |
|    | Celliton Blue Green B | 1.407 |

|    |                         |       |
|----|-------------------------|-------|
| 70 | Total class A dyestuffs | 9.936 |
|    | Fastusol Red L5B        | 6.156 |
|    | Fastusol Yellow 2 GA    | 2.638 |

|    |                         |        |
|----|-------------------------|--------|
| 75 | Total class B dyestuffs | 8.794  |
|    | Total dyestuffs         | 18.730 |

Similarly other shades are produced by preparing dye paste containing at least one dyestuff from each of the two classes.

Water and dye paste are mixed to prepare a dye bath of suitable dyeing level, as can be readily determined by those skilled in the art. Ordinarily about 80 parts of water to 1 part by weight of Panama hats has been found satisfactory.

An emulsifying agent is also added to the dye bath. The exact amount depends upon the nature of the emulsifying agent, but is ordinarily about 5% of the weight of the palm fiber being dyed. The emulsifying agent is ordinarily a water solution containing about 5% of a commercial emulsifying chemical. Nekal NS and Peregol O have been found to be excellent emulsifying chemicals.

In preparing a dye bath for dyeing palm fiber canary yellow, the following proportions may be used:

|                       |     |        |
|-----------------------|-----|--------|
| Palm fiber            | gms | 990    |
| Dyestuffs (see above) | gms | 12.8   |
| Peregal (5% solution) | cc  | 50     |
| Water                 | cc  | 79,200 |

In preparing a dye bath for dyeing palm fiber roseleaf pink, the following proportions may be used:

|                       |     |        |
|-----------------------|-----|--------|
| Palm fiber            | gms | 685    |
| Dyestuffs (see above) | gms | 18.730 |
| Peregal (5% solution) | cc  | 34     |
| Water                 | cc  | 55,000 |

## DYEING PROCESS

The dyeing solution is heated to approximately 120° F. Then the palm fiber is introduced. The temperature of the dyeing solution is gradually raised to or near to the boiling point, normally within about twenty-five minutes, but preferably in not less than twenty nor more than thirty minutes. The dyeing solution is then maintained at the high temperature, most conveniently at the boiling point, which is normally about 212° F., until the desired penetration of the dye is achieved. Keeping the dyeing solution at the boiling point for an hour has been found to give satisfactory penetration, but the period necessarily varies with the condition of the palm fiber, the shade being dyed, and other factors.

The dyeing solution is then drained from the hats, and the hats are allowed to dry. Although any suitable drying means is effective, it has been found that permitting the hats to dry under normal room conditions is quite satisfactory and the most economical method of drying.

## LACQUERING

Although the dried and dyed hats have the same shade upon the bruised and unbruised spots, the light reflects from the respective portions differently. It has been found that by the use of suitable lacquers it is possible to develop a uniform reflection of light from the entire hat. In the past uniform reflection of light from the bruised and unbruised portions has been achieved partly by means of the sulfur treatment.

In some instances hats dyed in the A-B dye bath of the present invention will not only have uniform shading but will also have uniform reflection characteristics. If uniform reflection characteristics are not produced in dyeing some certain shade, however, the nonuniform reflection may be taken care of by means of a lacquer developed by the present invention. According

to the present invention the reflection characteristics of any Panama hat may be improved by the application of a uniform reflection lacquer. According to the present invention, incorporating synthetic resins having suitable reflective and refractive properties, in a lacquer produces a uniform reflection lacquer. A lacquer which has been found satisfactory for imparting uniform reflection to a dyed palm fiber is:

DuPont methacrylate resin #2984

|                                | part by volume | 1 |
|--------------------------------|----------------|---|
| Hat thinner P & S #407         | parts          | 2 |
| Hat sizing lacquer P & S #8068 | do             | 4 |
| Lacquer thinner P & S #B5264   | do             | 8 |

In the above formula "P & S" refers to Pierce and Stevens of Buffalo, New York.

and Stevens, of Buffalo, New York.

While the exact formulas of the three Pierce and Stevens compositions are not obtainable, it is believed that similar compositions would have the following formulas:

*Hat thinner P & S #407*

|                                 | Parts |
|---------------------------------|-------|
| Isopropyl alcohol               | 1.5   |
| Normal butyl alcohol            | 1     |
| Hydrogenated naphtha            | 6     |
| Toluene                         | 6     |
| Ethylene glycol monoethyl ether | 6     |

Hat sizing lacquer P & S #8068

|                                           | Parts |
|-------------------------------------------|-------|
| 5 second nitrocellulose                   | 10    |
| Cellulose ethyl ether                     | 10    |
| Damar                                     | 3     |
| Tri beta monochlorethyl phosphate         | 2     |
| Bretylether condensate of dimethylol urea | 2     |
| Ethylene glycol monoethyl ether           | 61    |
| Toluene                                   | 63    |
| Hydrogenated naphtha                      | 61    |
| Normal butyl alcohol                      | 10    |
| Isopropyl alcohol                         | 15    |

LACQUER THINNER P & S #B5264

|                                 | Parts |
|---------------------------------|-------|
| Isopropyl alcohol               | 2     |
| Normal butyl alcohol            | 1     |
| Hydrogenated naphtha            | 6     |
| Toluene                         | 6     |
| Ethylene glycol monoethyl ether | 1     |

It will be understood that Du Pont methacrylate resin #2984 is monomethylmethacrylate. When the latter is resorted to, the hat is preferably given a preliminary coating of the lacquer by dipping in a lacquer such as given above. Then the hat is dummy blocked, and dipped in the lacquer again. The final pressing follows the second dipping. Preferably the hats are left untrimmed until after the second dipping in the lacquer.

Preferably a waterproofing component is incorporated in the lacquer. It has been found that Panama hats having been treated with a waterproofing agent are much more resistant to rain, and adverse weather conditions. Other suitable waterproofing agents of the well known class of waterproofing agents used on cotton or other cellulosic material may be used for this purpose. Methacrylate resin is a good waterproofing agent, and is incorporated in the above lacquer formula not only because of its uniform reflection properties but also because it functions as a waterproofing agent.

## PRODUCT

The process of the present invention produces  
75 dyed material having substantially the physical

properties of undyed material, and having substantially complete and uniform penetration of the dye. The product possesses substantially the same shade upon both the bruised and unbruised portions of the fiber. Light is reflected substantially uniformly from the entire product because the lacquer coating covers up the differences in reflection which would otherwise be produced by the bruised and unbruised fibers. The palm fibers are resistant to water by reason of being coated with a lacquer containing a water-proofing agent.

Dyed palm fiber contains the reaction product of the dyes used in the dyeing process. Because the reaction product cannot be named with perfect accuracy, it is sometimes hereinafter designated as the dyestuff. The product of the present invention is palm fiber containing at least one of each of class A dyestuffs, and class B dyestuffs. Panama hats made in accordance with the process of the present invention meet all of the commercial requirements of freedom from fading, weather resistance, strength, etc.

Parts of the present invention may be used without others. Many modifications of the process and product are possible without departing from the spirit of the present invention as described in this specification.

What is claimed as new is:

1. The process of dyeing slightly bruised sulfur-free Panama hats comprising the steps of: preparing a dyeing solution containing water, an emulsifying agent, at least one dyestuff chosen from the class consisting of acetate dyestuffs, and oil or spirit soluble dyestuffs, and at least one dyestuff chosen from the class consisting of direct dyestuffs, and neutral dyeing acid dyestuffs; penetratingly wetting out the Panama hats; and placing the wetted fibers in the dyeing solution.

2. The process of dyeing slightly bruised sulfur-free Panama hats comprising the steps of: preparing a dyeing solution containing water, an emulsifying agent, at least one dyestuff chosen from the class consisting of acetate dyestuffs, and oil or spirit soluble dyestuffs, and at least one dyestuff chosen from the class consisting of direct dyestuffs, and neutral dyeing acid dyestuffs; penetratingly wetting out the Panama hats; placing the wetted hats in the dyeing solution at a temperature of approximately 120° F.; gradually raising the temperature of the dyeing solution to about the boiling point; maintaining the dyeing solution at about the boiling point for about an hour; and withdrawing the palm fibers from the dyeing solution.

3. The process of dyeing slightly bruised sul-

fur-free bleached Panama hats comprising the steps of: preparing a dyeing solution containing water, an emulsifying agent, at least one dyestuff chosen from the class consisting of acetate dyestuffs, and oil or spirit soluble dyestuffs, and at least one dyestuff chosen from the class consisting of direct dyestuffs, and neutral dyeing acid dyestuffs; penetratingly wetting out the Panama hats in water at a temperature of approximately 60° F. for about twelve hours; placing the wetted hats in the dyeing solution at a temperature of approximately 120° F.; raising the temperature of the dyeing solution to about the boiling point within about twenty-five minutes; maintaining the dyeing solution at the boiling point for about an hour; and then withdrawing the hats from the dyeing solution.

4. The process of dyeing slightly bruised sulfur-free, untrimmed, bleached Panama hat bodies comprising the steps of: preparing a dyeing solution containing water, an emulsifying agent, at least one dyestuff chosen from the class consisting of acetate dyestuffs, and oil or spirit soluble dyestuffs, and at least one dyestuff chosen from the class consisting of direct dyestuffs, and neutral dyeing acid dyestuffs; penetratingly wetting out the hat bodies in a .1 per cent solution of a powerful wetting agent at 100° F. for five hours; placing the wetted hat bodies in the dyeing solution at a temperature of approximately 120° F.; raising the temperature of the dyeing solution to about the boiling point within about twenty-five minutes; maintaining the dyeing solution at about the boiling point for about an hour; and thereafter withdrawing the hat bodies from the dyeing solution.

5. An article formed from woven palm fibers dyed in substantially level shades with at least one dyestuff chosen from the class consisting of acetate dyestuffs, and oil or spirit soluble dyestuffs, and at least one dyestuff chosen from the class consisting of direct dyestuffs and neutral dyeing acid dyestuffs.

6. An article as defined in claim 5 having a coating of lacquer thereover to provide the dyed palm fibers with a uniform light-reflecting surface.

7. A palm fiber dyed in substantial level shades with at least one dyestuff chosen from the class consisting of acetate dyestuffs, and oil or spirit soluble dyestuffs, and at least one dyestuff chosen from the class consisting of direct dyestuffs and neutral dyeing acid dyestuffs.

GEORGE M. RICKUS.  
WILLIAM L. BRAUN.  
STANLEY G. HOFFMAN.